# EUROPEAN PATENT SPECIFICATION

(11) **EP 3 751 015 B1**
(45) Date of publication and mention of the grant of the patent: **20.04.2022**
(21) Application number: 20165731.9
(22) Date of filing: 25.03.2020
(51) Int. Cl.: C22C 1/10, C22C 32/00, C22C 1/05, C22C 9/00, C22C 29/08

(54) **PREPARATION METHOD OF A CU-NANO WC COMPOSITE MATERIAL**
HERSTELLUNGSVERFAHREN EINES CU-NANO WC-VERBUNDMATERIALS
MÉTHODE DE PRÉPARATION D'UN MATÉRIAU COMPOSITE CU-NANO WC

(30) Priority: 12.06.2019 CN 201910507514
(43) Date of publication of application: 16.12.2020
(73) Proprietor: Shaanxi Sirui Advanced Materials Co., Ltd., 710077 Xi'an Shaanxi (CN)
(72) Inventor: Wang, Wenbin, Xi'an Shaanxi 710077 (CN); Wang, Xiaojun, Xi'an Shaanxi 710077 (CN); Zhang, Shisong, Xi'an Shaanxi 710077 (CN); Liu, Kai, Xi'an Shaanxi 710077 (CN); LI, Peng, Xi'an Shaanxi 710077 (CN); Yang, Bin, Xi'an Shaanxi 710077 (CN); SHI, Xiaoyun, Xi'an Shaanxi 710077 (CN); Zhao, Jun, Xi'an Shaanxi 710077 (CN); LI, Gang, Xi'an Shaanxi 710077 (CN)
(74) Representative: Gong, Jinping

(56) References cited:
- YAO GONGCHENG ET AL: "High-performance copper reinforced with dispersed nanoparticles", JOURNAL OF MATERIALS SCIENCE, KLUWER ACADEMIC PUBLISHERS, DORDRECHT, vol. 54, no. 5, 26 November 2018 (2018-11-26), pages 4423-4432, XP036709861, ISSN: 0022-2461, DOI: 10.1007/S10853-018-3152-0 [retrieved on 2018-11-26]
- Srinath Viswanathan ET AL: "Vacuum Induction Melting" In: "ASM Handbook; Volume 15 Casting", 1 December 2008 (2008-12-01), ASM International, XP055694695, pages 116-123, DOI: 10.1361/asmhba0005200, * page 116; "process description" * * page 118, right column, 2nd paragraph * * figure 2 *

## Description

### TECHNICAL FIELD

The disclosure relates to the technical field of alloy material preparation, and particularly to a preparation method of a novel Cu-nano WC composite material.

### BACKGROUND

At present, the Cu-WC material is prepared by widely adopting a ceramimetallurgical manner due to limitation from difference in melting points and other properties of Cu and WC two materials. The Cu-WC material prepared by the ceramimetallurgical manner is low in density, high in gas content and low in conductivity, and the ceramimetallurgical manner cannot be used for preparing a composite material having WC content of 50% or below, thereby greatly limiting the application field of Cu-WC materials.

The preparation process in the prior art is as follows:

Powder mixing: WC powder and powder mixed with a small amount of Cu powder and other added members are uniformly mixed through powder mixing equipment;

Pressing: the uniformly mixed powder is pressed through pressing equipment to obtain a green body with certain binding strength and porosity;

Sintering a skeleton: the pressed green body is sintered at a protective atmosphere or in vacuum to prepare an infiltrated skeleton;

Infiltration: liquid Cu is infiltrated into the sintered WC skeleton at a temperature larger than a melting point of Cu in vacuum.

The vacuum infiltration method is a powder metallurgy process. The prepared Cu-WC has low density and high gas content. Because the skeleton needs to be sintered, the WC particle is relatively large in size, and the WC content must be >50%, and thus its conductivity is relatively low.

Based on the above existing problems, the disclosure has developed a Cu-WC material prepared by utilizing a vacuum induction melting method. The prepared Cu-WC material has low gas content and the vacuum induction melting method is suitable for preparing the Cu-WC composite material having WC content of ≤ 50%. Due to a cast structure, the Cu-WC material has a density of nearly 100%. The raw material adopts nano WC powder, so the strength of the material can be greatly improved through a nano strengthening effect.

YAO GONGCHENG ET AL: "High-performance copper reinforced with dispersed nanoparticles", Journal of Materials Science, Kluwer Academic Publishers, DORDRECHT, Vol. 54, No. 5, 26 November 2018, pages 4423-4432 describes a high performance copper based material and its producing method. Srinath Viswanathan ET AL: "Vacuum Induction Melting" in "ASM Handbook"; Volume 15 Casting ", 1 December 2008, ASM International, mentions the process of vacuum induction melting.

### SUMMARY

The technical problem to be solved by the disclosure is that the Cu-WC composite material prepared by the exiting technology is low in density, high in gas content and low in conductivity, and the composite material having WC content of 50% or below cannot be prepared, thereby greatly limiting the application field of Cu-WC materials.

The technical solution of the present invention is specified in independent claim 1.

A preparation method of a novel Cu-nano WC composite material, wherein the Cu-nano WC composite material meets the following conditions:
in a weight ratio, Cu powder: WC powder =98:2~30:70;
the Cu powder is of -200 meshes and has a purify of ≥99.7%, and the WC powder is 500 nano and has a purity of ≥99.0%;
the process comprises the following steps:
   S1) powder mixing process: Cu powder and WC are mixed in the above ratio and then the obtained mixed powder and steel balls are mixed for 3-10h in a weight ratio of mixed powder to steel balls of 100:100;
   S2) loose sintering process: the uniformly mixed powder is loosened into a graphite crucible and subsequently subjected to vacuum sintering; the obtained product is preserved for 2h at 950-1050°C when a vacuum degree reaches 5 × 10⁻² pa level or below so as to complete sintering, thereby obtaining a Cu-nano WC body; the raw materials are easy to form at the temperature of 950-1050°C, or else, they are difficultly sintered together if the temperature is low.
   S3) burdening process: the Cu-nano WC body subjected to loose sintering and oxygen-free Cu blocks are burdened in a weight ratio of Cu to WC of 99:1∼50:50; 50% of WC content is limit of the vacuum induction melting process; this ratio range can reach the effects of high temperature, high conductivity, wear resistance and low gas content;
   S4) vacuum induction melting process: the prepared Cu-nano WC body and the oxygen-free Cu blocks are put in a ceramic crucible, a vacuum system of vacuum induction melting equipment is switched on, the above reactants are subjected to gradient heating when the vacuum degree reaches 3 × 10⁻¹ pa or below, the specific gradient heating process is as follows: 10-20 KW, 1-5 min; 20-30 KW, 1-5 min; 30-40 KW, 1-5 min; 40-50 KW, 1-5 min; subsequently, power is kept at 40-60kw, when the oxygen-free Cu blocks are gradually molten in the crucible, the vacuum system is switched off, an inert protective gas is charged until the vacuum degree is -0.1~0.01 Mpa;
   S5) cooling process: after all the Cu-nano WC bodies in the crucible are completely dissolved by liquid Cu and are uniform under the action of electromagnetic stirring, the molten liquid in the crucible is poured into a cooling mould to be cooled for 1 h.

According to the preparation method of the disclosure, preferably, the particle size of the used steel ball in the process of powder mixing is 5-20 mm, and the rotation speed of the powder mixing machine is 10-30 r/min.

According to the preparation method of the disclosure, preferably, the electromagnetic stirring frequency is 1000-3000 Hz.

According to the preparation method of the disclosure, preferably, the cooling manner is water cooling.

According to the preparation method of the disclosure, preferably, the material of the cooling mould is chromium-copper alloy, water is introduced into the outside of the mould for heat conduction, and the water flow direction is from bottom to top.

The disclosure has the beneficial effects:
First, in the preparation method of the disclosure, Cu is added twice, the first addition of Cu is to ensure that the Cu-nano WC body is easy to form and degas in the process of loose sintering, and to facilitate the uniform dispersion of WC and Cu in the process of subsequent vacuum induction melting. The second addition of copper blocks is to gradually dissolve the Cu-nano WC body undergoing loose sintering utilizing the feature of first melting caused by low melting point of copper blocks, and finally uniformly disperse Cu and nano WC without agglomeration.
Second, the Cu-nano WC composite copper alloy material is prepared by the process of first powder mixing, then loose sintering, and then adding oxygen-free copper blocks for vacuum induction melting; this process is suitable for application occasions where the WC content is less than 50% compared with the process of "mixing powder, pressing, sintering skeleton and infiltration" in the prior art; this process utilizes the nano strengthening technology and does not need a large amount of addition, and thus the conductivity is relatively high, and the gas content of the vacuum induction melting material is low. Because of the cast structure, the Cu-nano WC composite copper alloy material has a density of nearly 100%. And the raw material uses nano WC powder, so the strength of the material can be greatly improved through the nano strengthening effect.

### DESCRIPTION OF THE EMBODIMENTS

The disclosure will be further described in combination with embodiments, but the protective scope of the disclosure is not limited thereto.

### <Cu-nano WC composite material>

The Cu-nano WC composite material of the disclosure meets the following conditions:
in a weight ratio, Cu powder: WC powder =98:2~30:70;
the Cu powder is of -200 meshes and has a purify of ≥99.7%, and the WC powder is <500 nano and has a purity of ≥99.0%;

### <preparation process of Cu-nano WC composite material>

The preparation process of the Cu-nano WC composite material of the disclosure comprises: powder mixing process S1), loose sintering process S2), burdening process S3), vacuum induction melting process S4) and cooling process S5).

### <power mixing process S1)>

The preparation process of the disclosure comprises the powder mixing process S1). In order that the uniformity of powder mixing is facilitated, the subsequent sintering is easy to exhaust and form and the uniformity of components of the final smelting process is facilitated, the powder mixing process S1) of the disclosure comprises:
S1) powder mixing process: the copper powder and WC are mixed in a weight ratio of Cu powder to WC powder of 98:2~30:70, and the mixed powder and steel balls are mixed for 3-10 h in a weight ratio of mixed powder to steel balls of 100:100.

### <loose sintering process S2)>

The preparation method of the disclosure comprises the loose sintering process S2). Because the materials are easily formed at the temperature of 950-1050 °C, or else they are difficultly sintered together due to low temperature; therefore, the loose sintering process S2) of the disclosure is as follows: the uniformly mixed powder is loosened into a graphite crucible, and then subjected to vacuum sintering. When the vacuum degree reaches 5 × 10⁻² pa level or below, the above product is preserved for 2 h at 950-1050 °C to obtain a Cu-nano WC body;

### <burdening process S3) >

The preparation method of the disclosure comprises a burdening process S3). In order to achieve the effect of high temperature, high conductivity, wear resistance and low gas content, the burdening process S3) of the disclosure comprises the following steps: the Cu-nano WC body subjected to loose sintering and free-oxygen copper blocks are burdened in a weight ratio of Cu to WC of 99:1∼50:50;

### < vacuum induction melting process S4) >

The preparation method of the disclosure comprises the vacuum induction smelting process S4). In the preparation method of the disclosure, cupper is added twice, first addition of cupper powder is to ensure that the Cu-nano WC body is easy to form and degas in the process of loose sintering and the uniform dispersion of WC and Cu is facilitated in the process of subsequent vacuum induction sintering, second addition of cupper blocks is to allow cupper blocks to be gradually molten to dissolve the Cu-nano WC body subjected to loose sintering by utilizing the characteristic that the cupper blocks are molten firstly due to low melting point and then to finally uniformly disperse Cu and nano WC without agglomeration; therefore, the vacuum induction melting process S4) of the disclosure is as follows: the prepared Cu-nano WC body and the free-oxygen copper blocks are put into the ceramic crucible, the vacuum system of the vacuum induction melting equipment is switched on, and the reactants are subjected to gradient heating when the vacuum degree reaches 3 × 10⁻¹ pa or below, and the specific process of gradient heating is: 10-20 KW, 1-5 min; 20-30 KW, 1-5 min; 30-40 KW, 1-5 min; 40-50 KW, 1-5 min; subsequently, the power is kept at 40-60kw, when the oxygen-free copper blocks in the crucible are gradually molten, the vacuum system is switched off, and the inert protective gas is charged until the vacuum degree is - 0.1 ~ 0.01 Mpa;

### < cooling process S5) >

The preparation process of the disclosure also comprises the cooling process S5): after all the Cu-nano WC bodies in the crucible are dissolved by liquid Cu, and are uniformly stirred under the action of an electromagnetic force, the molten liquid in the crucible is poured into a cooling mold to be cooled for 1 h.

### Example 1: preparation of CuWC4

Copper powder (- 200 meshes) having a purity ≥ 99.7% and WC (< 500 nm) having purity of ≥ 99.0% were selected as raw materials. First, copper powder and WC were mixed in a weight ratio of Cu powder to WC powder of 75:25, and then mixed for 3 h in a weight ratio of mixed powder to steel balls of 100:100; the diameter of the steel ball was 5 mm, and the rotation speed of a powder mixing machine was 10 r/min;
when the uniformly mixed powder was loosened into the graphite crucible and subsequently subjected to vacuum sintering, and when the vacuum degree was 5 × 10⁻² pa or below, the obtained product was preserved for 2h at 950 °C to complete sintering so as to obtain a Cu-nano WC body;
the Cu-nano WC body subjected to loose sintering and oxygen-free cupper blocks were burdened in a weight ratio of Cu to WC of 96:4;
the prepared Cu-nano WC body and oxygen-free copper blocks were put into the ceramic crucible, the vacuum system of the vacuum induction smelting equipment was switched on, and the reactants were subjected to gradient heating when the vacuum degree reached below 3 × 10⁻¹pa: 10 KW, 1 min; 20 KW, 1 min; 30 KW, 1min; 40 KW, 1 min; then the power was kept at 40 KW; when the oxygen-free copper blocks in the crucible were molten gradually, the vacuum system was switched off, and the inert protective gas was charged until the vacuum degree was -0.1 Mpa;

When all the Cu-nano WC bodies in the crucible were dissolved by liquid Cu and uniformly stirred under the action of an electromagnetic force at the frequency of 3000 Hz, then the molten liquid in the crucible was poured into the cooling mould to be subjected to water cooling for 1 h. The material of the cooling mould was low chromium copper alloy, and water was charged into the outside of the mold for heat conduction, and the water flow direction was from top to bottom.

### Example 2: preparation of CuWC6

Copper powder (- 200 meshes) having a purity of ≥ 99.7% and WC (< 500 nm) having a purity of ≥ 99.0% were selected as raw materials. First, copper powder and WC were mixed in a weight ratio of Cu powder to WC powder of 90:10, and then mixed for 5 h in a weight ratio of mixed powder to steel balls of 100:100; the diameter of the steel ball was 12 mm, and the rotation speed of a powder mixing machine was 13 r/min;
when the uniformly mixed powder was loosened into the graphite crucible and subsequently subjected to vacuum sintering, when the vacuum degree was 5 × 10⁻² pa or below, the obtained prodcut was preserved for 2 h at 980 °C to complete sintering so as to obtain a Cu-nano WC body;
the Cu-nano WC body subjected to loose sintering and oxygen-free cupper blocks were burdened in a weight ratio of Cu to WC of 94:6;
the prepared Cu-nano WC body and oxygen-free copper blocks were put into the ceramic crucible, the vacuum system of the vacuum induction smelting equipment was switched on, and the reactants were subjected to gradient heating when the vacuum degree reached below 3 × 10⁻¹ pa: 12 KW, 2 min; 24 KW, 2 min; 33 KW, 3 min; 42 KW, 2 min; subsequently, the power was kept at 46 KW; when the oxygen-free copper blocks in the crucible were molten gradually, the vacuum system was switched off, and the inert protective gas was charged until the vacuum degree was - 0.06 Mpa;

When all the Cu-nano WC bodies in the crucible were dissolved by liquid Cu and uniformly stirred under the action of an electromagnetic force at the frequency of 2400 Hz, then the molten liquid in the crucible was poured into the cooling mould to be subjected to water cooling for 1h. The material of the cooling mold was low chromium copper alloy, and water was charged into the outside of the mould for heat conduction, and the water flow direction was from top to bottom.

### Example 3 preparation of CuWC8

Copper powder (- 200 meshes) having a purity of ≥ 99.7% and WC (< 500 nm) having a purity of ≥ 99.0% were selected as raw materials. First, copper powder and WC were mixed in a weight ratio of Cu powder to WC powder of 80:20, and then mixed for 5 h in a weight ratio of mixed powder to steel ball of 100:100; the diameter of the steel ball was 16 mm, and the rotation speed of a powder mixing machine was 22 r/min;
when the uniformly mixed powder was loosened into the graphite crucible and subsequently subjected to vacuum sintering, when the vacuum degree was 5 × 10⁻² pa or below, the obtained product was preserved for 2h at 1000 °C to complete sintering so as to obtain a Cu-nano WC body;
the Cu-nano WC body subjected to loose sintering and oxygen-free cupper blocks were burdened in a weight ratio of Cu to WC of 92:8;
the prepared Cu-nano WC body and oxygen-free copper blocks were put into the ceramic crucible, the vacuum system of the vacuum induction smelting equipment was switched on, and the reactants were subjected to gradient heating when the vacuum degree reached below 3 × 10⁻¹ pa: 18 KW, 5 min; 26 KW, 3 min; 35 KW, 4 min; 45 KW, 3 min; then the power was kept at 48 KW; when the oxygen-free copper blocks in the crucible were molten gradually, the vacuum system was switched off, and the inert protective gas was charged until the vacuum degree was -0.05 Mpa;

When all the Cu-nano WC bodies in the crucible were dissolved by liquid Cu and uniformly stirred under the action of an electromagnetic force at the frequency of 1900 Hz, then the molten liquid in the crucible was poured into the cooling mould to be subjected to water cooling for 1 h. The material of the cooling mould was low chromium copper alloy, and water was charged into the outside of the mould for heat conduction, and the water flow direction was from top to bottom.

### Example 4 preparation of CuWC30

Copper powder (- 200 meshes) having a purity of ≥ 99.7% and WC (< 500 nm) having a purityof ≥ 99.0% were selected as raw materials. First, copper powder and WC were mixed in a weight ratio of Cu powder to WC powder of 40:60, and then mixed for 8 h in a weight ratio of mixed powder to steel balls of 100:100; the diameter of the steel ball was 20 mm, and the rotation speed of a powder mixing machine was 25 r/min;
when the uniformly mixed powder was loosened into the graphite crucible and subsequently subjected to vacuum sintering, when the vacuum degree was 5 × 10⁻² pa or below, the obtained product was preserved for 2 h at 1020 °C to complete sintering so as to obtain a Cu-nano WC body;
the Cu-nano WC body subjected to loose sintering and oxygen-free cupper blocks were burdened in a weight ratio of Cu to WC of 70:30;
the prepared Cu-nano WC body and oxygen-free copper blocks were put into the ceramic crucible, the vacuum system of the vacuum induction smelting equipment was switched on, and the reactants were subjected to gradient heating when the vacuum degree reached below 3 × 10⁻¹ pa: 18 KW, 4 min; 22 KW, 5 min; 37 KW, 5 min; 50 KW, 5 min; then the power was kept at 50kW; when the oxygen-free copper blocks in the crucible were molten gradually, the vacuum system was switched off, and the inert protective gas was charged until the vacuum degree was -0.01 Mpa;

When all the Cu-nano WC bodies in the crucible were dissolved by liquid Cu and uniformly stirred under the action of an electromagnetic force at the frequency of 1500 Hz, and then the molten liquid in the crucible was poured into the cooling mould to be subjected to water cooling for 1 h. The material of the cooling mould was low chromium copper alloy, and water was charged into the outside of the mould for heat conduction, and the water flow direction was from top to bottom.

### Example 5 preparation of CuWC35

Copper powder (- 200 meshes) having a purity of ≥ 99.7% and WC (< 500 nm) having a purity of ≥ 99.0% were selected as raw materials. First, copper powder and WC were mixed in a weight ratio of Cu powder to WC powder of 50:50, and then mixed for 9 h in a weight ratio of mixed powder to steel ball of 100:100; the diameter of the steel ball was 18 mm, and the rotation speed of a powder mixing machine was 24 r/min;
when the uniformly mixed powder was loosened into the graphite crucible and subsequently subjected to vacuum sintering, when the vacuum degree was 5 × 10⁻² pa or below, the obtained product was preserved for 2 h at 1050 °C to complete sintering so as to obtain a Cu-nano WC body;
the Cu-nano WC body subjected to loose sintering and oxygen-free cupper blocks were burdened in a weight ratio of Cu to WC of 65:35;
the prepared Cu-nano WC body and oxygen-free copper blocks were put into the ceramic crucible, the vacuum system of the vacuum induction smelting equipment was switched on and the reactants were subjected to gradient heating when the vacuum degree reached below 3 × 10⁻¹ pa: 20 KW, 5 min; 20 KW, 2 min; 30 KW, 1 min; 40 KW, 1 min; then the power was kept at 42 KW; when the oxygen-free copper blocks in the crucible were molten gradually, the vacuum system was switched off, and the inert protective gas was charged until the vacuum degree was 0.01 Mpa;

When all the Cu-nano WC bodies in the crucible were dissolved by liquid Cu and uniformly stirred under the action of an electromagnetic force at the frequency of 1300 Hz, then the molten liquid in the crucible was poured into the cooling mould to be subjected to water cooling for 1 h. The material of the cooling mould was low chromium copper alloy, and water was charged into the outside of the mould for heat conduction, and the water flow direction was from top to bottom.

### Example 6 preparation of CuWC50

Copper powder (- 200 meshes) having a purity of ≥ 99.7% and WC (< 500 nm) having a purity of ≥ 99.0% were selected as raw materials. First, copper powder and WC were mixed in a weight ratio of Cu powder to WC powder of 30:70, and then mixed for 10 h in a weight ratio of mixed powder to steel balls of 100:100; the diameter of the steel ball was 19 mm, and the rotation speed of a powder mixing machine was 26 r/min;
when the uniformly mixed powder was loosened into the graphite crucible and subsequently subjected to vacuum sintering, when the vacuum degree was 5 × 10⁻² pa or below, the obtained product was preserved for 2 h at 1050 °C to complete sintering so as to obtain a Cu-nano WC body;
th Cu-nano WC body subjected to loose sintering and oxygen-free cupper blocks were burdened in a weight ratio of Cu to WC of 50:50;
the prepared Cu-nano WC body and oxygen-free copper blocks were put into the ceramic crucible, the vacuum system of the vacuum induction smelting equipment was switched on, and the reactants were subjected to gradient heating when the vacuum degree reached below 3 × 10⁻¹ pa: 20 KW, 5 min; 22 KW, 4 min; 40 KW, 5 min; 41 KW, 5 min; then the power was kept at 60kW; when the oxygen-free copper blocks in the crucible were molten gradually, the vacuum system was switched off, and the inert protective gas was charged until the vacuum degree was -0.01 Mpa;

When all the Cu-nano WC bodies in the crucible were dissolved by liquid Cu and uniformly stirred under the action of an electromagnetic force at the frequency of 1000 Hz, then the molten liquid in the crucible was poured into the cooling mould to be subjected to water cooling for 1 h. The material of the cooling mould was low chromium copper alloy, and water was charged into the outside of the mould for heat conduction, and the water flow direction was from top to bottom.

Various property parameters of Cu-nano WC composite cupper alloy materials prepared in the above examples 1-6 are shown in Table 1.

**Table 1: Table of property parameters of various models of Cu-nano WC composite cupper alloy materials in examples 1-6**

| Group | Name | WC content % | Cu content % | Vacuum sintering temperature °C | Oxygen content ppm | Nitrogen content ppm | Conductivity MS/m | Hardness (cast) HB | Hardness (900°C annealing) HB |
|---|---|---|---|---|---|---|---|---|---|
| Example 1 | CuWC4 | 4 | Residue | 950 | <20 | <20 | >52 | 58-70 | 58-70 |
| Example 2 | CuWC6 | 6 | Residue | 980 | <30 | <20 | >49 | 63-75 | 63-75 |
| Example 3 | CuWC8 | 8 | Residue | 1000 | <40 | <20 | >45 | 70-85 | 70-85 |
| Example 4 | CuWC30 | 30 | Residue | 1020 | <100 | <50 | >37 | 190-220 | 190-220 |
| Example 5 | CuWC35 | 35 | Residue | 1050 | <120 | <50 | >33 | 220-240 | 220-240 |
| Example 6 | CuWC50 | 50 | Residue | 1050 | <150 | <50 | >25 | 270-300 | 270-300 |
| 900°C annealing without softness | | | | | | | | | |

It can be seen from the above data that the method of the disclosure can prepare the Cu-WC composite material having WC content of ≤50%, and the material is high in strength, low in gas content, high in conductivity and high in density, and has significant advantages compared with the prior art.

### Experimental example

### 1. Study on effect of a ratio of Cu powder to WC powder on properties of composite material

A powder mixing ratio where copper powder and WC were mixed in a weight ratio of Cu powder to WC powder of 99:1 was used as a comparative example 1, a powder mixing ratio where copper powder and WC were mixed in a weight ratio of Cu powder to WC powder of 28:72 was used as a comparative example 2, a powder mixing ratio where copper powder and WC were mixed in a weight ratio of Cu powder to WC powder of 90:10 was used as a comparative example 3, a powder mixing ratio where copper powder and WC were mixed in a weight ratio of Cu powder to WC powder of 80:20 was used as a comparative example 4, a powder mixing ratio where copper powder and WC were mixed in a weight ratio of Cu powder to WC powder of 50:50 was used as a comparative example 5, a powder mixing ratio where copper powder and WC were mixed in a weight ratio of Cu powder to WC powder of 40:60 was used as a comparative example 6, and various comparative examples performed preparation of composite materials according to the preparation method of example 1. In comparative example 1, oxygen-free cupper blocks were not added in step (3), and other parameters are the same as those in example 1 except that the ratio of Cu powder to WC powder when in primary powder mixing was different. The property parameters of the obtained composite material are shown in Table 2:

**Table 2: Table of property parameters of Cu-nano WC composite cupper alloy materials prepared in comparative examples 1-2**

| Group | Name | WC content % | Cu content % | Ratio of Cu powder to WC powder during the powder mixing | Oxygen content ppm | Nitrogen content ppm | Conductivity MS/m | Hardness (cast) HB | Hardness (900°C annealing ) HB |
|---|---|---|---|---|---|---|---|---|---|
| Comparative example 1 | CuWC1 | 1 | Residue | 99:1 | <150 | <150 | <20 | 8-20 | 8-20 |
| Comparative example 2 | CuWC4 | 4 | Residue | 28:72 | >160 | >40 | <45 | 35-66 | 35-66 |
| Comparative example 3 | CuWC4 | 4 | Residue | 90: 10 | <18 | <18 | >53 | 58-70 | 58-70 |
| Comparative example 4 | CuWC4 | 4 | Residue | 80: 20 | <10 | <10 | >56 | 62-80 | 62-80 |
| Comparative example 5 | CuWC4 | 4 | Residue | 50: 50 | <20 | <20 | >55 | 60-70 | 60-70 |
| Comparative example 6 | CuWC4 | 4 | Residue | 40: 60 | <20 | <20 | >53 | 58-73 | 58-73 |
| Example 1 | CuWC4 | 4 | Residue | 75:25 | <20 | <20 | >52 | 58-70 | 58-70 |

It can be seen from the above data that when the ratio of Cu powder to WC powder is greater than 98:2 or less than 30:70 in the process of powder mixing, it is not conducive to uniform powder mixing, exhausting and forming, and is not conducive to the uniformity of components in the process of final smelting, thereby resulting in a fact that the prepared Cu-WC composite material is high in gas content, low in electrical conductivity and greatly reduced material strength and wear resistance, and does not meet the use requirement.

**Conclusion 1:** under the condition that all the parameters are the same (the main control parameters are: the melting ratio is Cu: WC = 96:4; the vacuum sintering temperature is 950 °C), when the mixing ratio of Cu powder to WC powder is 80:20, it is conducive to the uniform powder mixing, easy to exhaust and form in the next sintering, and is also conducive to the uniformity of components in the process of final smelting. The prepared composite material is low in gas content, and relatively high in material strength and hardness and conductivity.

### 2. Study on effect of vacuum sintering temperature on properties of composite material

930 °C vacuum sintering temperature was used as comparative example 7, 1080 °C vacuum sintering temperature was used as comparative example 8, 970 °C vacuum sintering temperature was used as comparative example 9, 1010 °C vacuum sintering temperature was used comparative example 10, and 1040 °C vacuum sintering temperature was used as comparative example 11. The composite material is prepared according to the preparation method of example 3. Other parameters were the same as those in example 3 except the vacuum sintering temperature was different. The property parameters of the obtained composite material are shown in Table 3:

**Table 3: Table of property parameters of Cu-nano WC composite copper alloy materials prepared in comparative examples 3-4**

| Group | Name | WC content % | Cu content % | Vacuum sintering temperature °C | Oxygen content ppm | Nitrogen content ppm | Conductivity MS/m | Hardness (cast) HB | Hardness (900°C annealing ) HB |
|---|---|---|---|---|---|---|---|---|---|
| Comparative example 7 | CuWC8 | 8 | Residue | 930 | <65 | <30 | >15 | 40-70 | 40-70 |
| Comparative example 8 | CuWC8 | 8 | Residue | 1080 | <50 | <30 | >12 | 45-73 | 45-73 |
| Comparative example 9 | CuWC8 | 8 | Residue | 970 | <40 | <30 | >45 | 72-85 | 72-85 |
| Comparative example 10 | CuWC8 | 8 | Residue | 1010 | <40 | <20 | >50 | 70-80 | 70-80 |
| Comparative example 11 | CuWC8 | 8 | Residue | 1040 | <40 | <20 | >48 | 70-80 | 70-80 |
| Example 3 | CuWC8 | 8 | Residue | 1000 | <40 | <20 | >45 | 70-85 | 70-85 |

It can be seen from the above data that when the vacuum sintering temperature is less than 950°C or greater than 1050 °C, relatively, the prepared Cu-WC composite material becomes high in gas content and becomes poor in conductivity, especially, when the temperature is less than 950°C, the material is not easy to form and is difficultly sintered together, so as to cause difficult subsequent smelting, resulting in greatly reduced strength and wear resistance of the material, which does not meet the use requirement. Thus, it is suitable to control the vacuum sintering temperature to be between 950°C and 1050°C, and the prepared material is good in various properties.

**Conclusion 2:** under the condition that all the parameters are the same (the main control parameters are: the ratio of Cu powder to WC powder is 80:20; when in smelting, Cu : WC is 92:8), when the vacuum sintering temperature is 1010°C, the material is easy to form and conducive to sintering, and it is also conducive to the uniformity of components in the process of final smelting. The prepared composite material is low in gas content, and relatively high in material strength and hardness and conductivity.

### 3. Study on effect of WC content on properties of composite material

Example 3 was used as reference, WC content of 0.8% was used as comparative example 12, WC content of 53 % was used as comparative example 13, WC content of 2% was used as comparative example 13, WC content of 15% was used as comparative example 15, WC content of 25% was used as a comparative example 16, and WC content of 50% was used as comparative example 17. The composite material was prepared according to the preparation method in example 3. Other parameters were the same as those in example 3 except the vacuum sintering temperature was different. The property parameters of the obtained composite materials are shown in Table 4:

**Table 4: Table of property parameters of Cu-nano WC composite copper alloy materials prepared in comparative examples 5-6**

| Group | Name | WC content % | Cu content % | Vacuum sintering temperature °C | Oxygen content ppm | Nitrogen content ppm | Conductivity MS/m | Hardness (cast) HB | Hardness (900°C annealing ) HB |
|---|---|---|---|---|---|---|---|---|---|
| Comparative example 12 | CuWC0.8 | 0.8 | Residue | <30 | <20 | >55 | 35-45 | 35-45 | <30 |
| Comparative example 13 | CuWC53 | 53 | Residue | <170 | <80 | >20 | 70-85 | 70-85 | <170 |
| Comparative example 14 | CuWC2 | 2 | Residue | <20 | <20 | >57 | 40-50 | 40-50 | <20 |
| Comparative example 15 | CuWC15 | 15 | Residue | <45 | <20 | >43 | 60-180 | 60-180 | <45 |
| Comparative example 16 | CuWC25 | 25 | Residue | <50 | <20 | >41 | 70-185 | 70-185 | <50 |
| Comparative example 17 | CuWC50 | 50 | | <140 | <40 | >32 | 150-185 | 150-185 | <140 |
| Example 3 | CuWC8 | 8 | Residue | <40 | <20 | >45 | 70-85 | 70-85 | <40 |

It can be seen from the above data that when the WC content is less than 1%, the prepared Cu-WC composite material has low gas content and high conductivity, but its material strength and wear resistance are greatly reduced. When the WC content is higher than 50%, the prepared Cu-WC composite material has good strength and wear resistance, but has high gas content and poor conductivity, so it does not meet the user requirement. Therefore, it is suitable to control the WC content within the range from 1% to 50%, and the prepared material is good in various properties.

**Conclusion 3:** under the condition that all the parameters are the same (the main control parameters are: when in powder mixing, Cu powder: WC powder = 80:20; vacuum sintering temperature is 1000 °C), when the WC content is 15%, the prepared composite material has excellent properties in the aspects of gas content, material strength, hardness and conductivity.

It is worth noting that those skilled in the art can directly derive or associate some deformations from the contents of the disclosure and common senses under the enlightenment of the concept and specific embodiments of the disclosure. Those of ordinary skill in the art will appreciate that other methods or the common known technologies in the prior art can be replaced, as well as different combinations of features and other non-substantive modifications can also be adopted. Similarly, the functions and effects described in the disclosure can also be realized, which are not described in detail one by one, and belong to the protective scope of the disclosure.

## Claims

1. A preparation method of a Cu-nano WC composite material, wherein the Cu-nano WC composite material meets the following conditions:
in a weight ratio, Cu powder: WC powder=98:2~30:70;
the Cu powder is of -200 meshes and has a purify of ≥99.7%, and the WC is <500 nano and has a purity of ≥99.0%;
the process comprises the following steps:
S1) powder mixing process: Cu powder and WC are mixed in the above ratio and then the obtained mixed powder and steel balls are mixed for 3-10 h in a weight ratio of mixed powder to steel balls of 100:100;
S2) loose sintering process: the uniformly mixed powder is loosened into a graphite crucible and subsequently subjected to vacuum sintering; when a vacuum degree reaches 5 × 10⁻² pa level or below, the obtained product is preserved for 2 h at 950-1050 °C so as to complete sintering, thereby obtaining a Cu-nano WC body;
S3) burdening process: the Cu-nano WC body subjected to loose sintering and oxygen-free Cu blocks are burdened in a weight ratio of Cu to WC of 99:1~50:50;
S4) vacuum induction melting process: the prepared Cu-nano WC body and the oxygen-free Cu blocks are put in a ceramic crucible, a vacuum system of vacuum induction melting equipment is opened, the above reactants are subjected to gradient heating when the vacuum degree reaches 3 × 10⁻¹ pa or below, the specific gradient heating process is as follows: 10-20 KW, 1-5 min; 20-30 KW, 1-5 min; 30-40 KW, 1-5 min; 40-50 KW, 1-5 min; subsequently, power is kept at 40-60kw, when the oxygen-free Cu blocks are gradually molten in the crucible, the vacuum system is switched off, an inert protective gas is charged until the vacuum degree is -0.1~0.01 Mpa;
S5) cooling process: after all the Cu-nano WC bodies in the crucible are completely dissolved by liquid Cu and are uniform under the action of electromagnetic stirring, the molten liquid in the crucible is poured into a cooling mould to be cooled for 1 h.

2. The preparation method of the Cu-nano WC composite material according to claim 1, wherein in the process of ball milling and powder mixing, the particle size of the used steel ball is 5-20 mm, and the rotation speed of a powder mixing machine is 10-30 r/min.

3. The preparation method of the Cu-nano WC composite material according to claim 1, wherein the electromagnetic stirring frequency is 1000-3000 Hz.

4. The preparation method of the Cu-nano WC composite material according to claim 1, wherein the cooling manner is water cooling.

5. The preparation method of the Cu-nano WC composite material according to claim 4, wherein the material of the cooling mould is chromium-copper alloy, water is introduced into the outside of the mould for heat conduction, and the water flow direction is from bottom to top.

## Patentansprüche

1. Verfahren zur Vorbereitung eines Cu-Nano-WC-Verbundmaterials, wobei das Cu-Nano-WC-Verbundmaterial die folgenden Bedingungen erfüllt:
in einem Gewichtsverhältnis Cu-Pulver: WC-Pulver=98:2 bis 30:70;
wobei das Cu-Pulver -200 Maschen und eine Reinheit von ≥99,7% aufweist, und wobei das WC <500 nano ist und eine Reinheit von ≥99,0% aufweist;
wobei das Verfahren die folgenden Schritte umfasst:
S1) Pulvermischverfahren: bei dem das Cu-Pulver und WC im oben genannten Verhältnis gemischt werden und dann das erhaltene gemischte Pulver und die Stahlkugeln für 3-10h in einem Gewichtsverhältnis von gemischtem Pulver zu Stahlkugeln von 100:100 gemischt werden;
S2) loses Sinterverfahren: bei dem das gleichmäßig gemischte Pulver in einem Graphittiegel aufgelockert und anschließend dem Vakuumsintem unterzogen wird, wobei das erhaltene Produkt für 2 Stunden bei 950-1050°C aufbewahrt wird, wenn ein Vakuumgrad einen Wert von 5 × 10⁻² pa oder darunter erreicht, sodass das Sintern vervollständigt wird, wodurch ein Cu-Nano-WC-Körper erhalten wird;
S3) Möllerverfahren: bei dem der Cu-Nano-WC-Körper, der einer losen Sinterung unterzogen wird, und die sauerstofffreien Cu-Blöcke in einem Gewichtsverhältnis von Cu zu WC von 99:1 bis 50:50 gemöllert werden;
S4) Vakuuminduktionsschmelzverfahren: bei dem der vorbereitete Cu-Nano-WC-Körper und die sauerstofffreien Cu-Blöcke in einen Keramiktiegel gegeben werden, wobei ein Vakuumsystem der Vakuuminduktionsschmelzanlage geöffnet wird, wobei die oben genannten Reaktanten einer Gradientenerwärmung unterzogen werden, wenn der Vakuumgrad 3 × 10⁻¹ pa oder weniger erreicht, wobei das spezifische Gradientenerwärmungsverfahren wie folgt ist: 10-20 KW, 1-5 min; 20-30 KW, 1-5 min; 30-40 KW, 1-5 min; 40-50 KW, 1-5 min; wobei die Leistung anschließend bei 40-60kw gehalten wird, wenn die sauerstofffreien Cu-Blöcke im Tiegel allmählich geschmolzen sind, wobei das Vakuumsystem ausgeschaltet wird, ein inertes Schutzgas eingefüllt wird, bis der Vakuumgrad -0,1~0,01 Mpa beträgt;
S5) Abkühlungsprozess: nachdem alle Cu-Nano-WC-Körper im Tiegel vollständig durch flüssiges Cu aufgelöst und unter der Einwirkung von elektromagnetischem Rühren homogenisiert werden, wird die geschmolzene Flüssigkeit im Tiegel in eine Kühlform gegossen und für 1 h abgekühlt.

2. Verfahren zur Vorbereitung des Cu-Nano-WC-Verbundmaterials nach Anspruch 1, wobei im Verfahren des Kugelmahlens und Pulvermischens die Teilchengröße der verwendeten Stahlkugel 5-20 mm beträgt und die Rotationsgeschwindigkeit einer Pulvermischmaschine 10-30 r/min beträgt.

3. Verfahren zur Vorbereitung des Cu-Nano-WC-Verbundmaterials nach Anspruch 1, wobei die elektromagnetische Rührfrequenz 1000-3000 Hz beträgt.

4. Verfahren zur Vorbereitung des Cu-Nano-WC-Verbundmaterials nach Anspruch 1, wobei die Kühlung mittels Wasser erfolgt.

5. Verfahren zur Vorbereitung des Cu-Nano-WC-Verbundmaterials nach Anspruch 4, wobei das Material der Kühlform eine Chrom-Kupfer-Legierung ist, wobei das Wasser zur Wärmeleitung in die Außenseite der Form eingeleitet wird und die Richtung des Wasserflusses von unten nach oben verläuft.

## Revendications

1. Un procédé de préparation d'un matériau composite Cu-nano WC, dans lequel le matériau composite Cu-nano WC satisfait aux conditions suivantes :
dans un rapport pondéral, Cu poudre: WC poudre=98:2-30:70;
la poudre de Cu est de -200 mailles et a une pureté de ≥99,7%, et le WC est <500 nano et a une pureté de ≥99,0%;
le procédé comprend les étapes suivantes:
S1) processus de mélange de poudre: la poudre de Cu et de WC sont mélangés dans le rapport ci-dessus, puis la poudre mélangée obtenue et les billes d'acier sont mélangées pendant 3-10 h dans un rapport pondéral de la poudre mélangée aux billes d'acier de 100:100;
S2) processus de frittage lâche: la poudre uniformément mélangée est relâchée dans un creuset en graphite et ensuite soumise à un frittage sous vide; lorsqu'un degré de vide atteint un niveau de 5 × 10⁻² pa ou moins, le produit obtenu est conservé pendant 2 h à 950-1050 °C afin d'achever le frittage, obtenant ainsi un corps Cu-nano WC;
S3) processus de charge: le corps Cu-nano WC soumis à un frittage lâche et des blocs de Cu sans oxygène sont chargés dans un rapport pondéral de Cu aux WC de 99:1-50:50;
S4) processus de fusion par induction sous vide: le corps Cu-nano WC préparé et les blocs de Cu sans oxygène sont placés dans un creuset en céramique, un système sous vide d'équipement de fusion par induction sous vide est ouvert, les réactifs ci-dessus sont soumis à un chauffage par gradient lorsque le vide degré atteint 3 × 10⁻¹ pa ou moins, le processus de chauffage par gradient spécifique est le suivant: 10-20 KW, 1-5 min; 20-30 KW, 1-5 min; 30-40 KW, 1-5 min; 40-50 KW, 1-5 min; ensuite, la puissance est maintenue à 40-60kw, lorsque les blocs de Cu sans oxygène fondent progressivement dans le creuset, le système de vide est éteint, un gaz protecteur inerte est chargé jusqu'à ce que le degré de vide soit de -0,1-0,01 Mpa;
S5) processus de refroidissement: après que tous les corps Cu-nano WC dans le creuset sont complètement dissous par le Cu liquide et sont uniformes sous l'action de l'agitation électromagnétique, le liquide fondu dans le creuset est versé dans un moule de refroidissement pour être refroidi pendant 1 h.

2. Le procédé de préparation du matériau composite Cu-nano WC selon la revendication 1, dans lequel, dans le processus de broyage à billes et de mélange de poudre, la taille des particules de la bille d'acier utilisée est de 5-20 mm, et la vitesse de rotation d'une machine de mélange de poudre est de 10-30 r/min.

3. Le procédé de préparation du matériau composite Cu-nano WC selon la revendication 1, dans lequel la fréquence d'agitation électromagnétique est de 1000-3000 Hz.

4. Le procédé de préparation du matériau composite Cu-nano WC selon la revendication 1, dans lequel la méthode de refroidissement est un refroidissement à l'eau.

5. Le procédé de préparation du matériau composite Cu-nano WC selon la revendication 4, dans lequel le matériau du moule de refroidissement est un alliage chrome-cuivre, de l'eau est introduite à l'extérieur du moule pour la conduction de la chaleur, et la direction d'écoulement de l'eau est du bas en haut.
